

# United States Patent Office

3,186,926

Patented June 1, 1965

1

3,186,926  
ELECTROPLATING SOLUTION CONTAINING A  
DIESTER OF SELENIOUS ACID  
Hans Hofmann, Neuss (Rhine), Germany (Gustav Klein  
Strasse 8, Stuttgart-Feuerbach, Germany), and Karl  
Wilhelm Sassenroth, Dusseldorf, Germany (Room-  
strasse 65, Bielefeld, Germany)  
No Drawing. Filed Aug. 13, 1962, Ser. No. 216,317  
9 Claims. (Cl. 204—49)

This invention relates to electrolytic deposition of bright metal coatings using electroplating baths to which brighteners are added. It is already known that additions of selenium compounds, preferably selenious acid or salts thereof, are active as brighteners in various electroplating baths.

Thus, it has already been proposed, a relatively long time ago, to use selenious acid and salts thereof as additives, together with an albumen condensation product, for silver baths for the production of bright silver coatings. Recently, it has also been proposed to use selenious acid in combination with various wetting agents in copper baths, as a brightener. Selenium dioxide is also known as an active brightener in nickel baths, and selenium compounds, namely selenium dithiocarbamate, and selenium in a form providing divalent negative ions have also already been proposed as additives for silver, gold and copper-plating baths.

We have found, unexpectedly, that selenium in the form of its very readily accessible selenious acid ester together with alcohols, phenols, thiophenols and thioalcohols, when used as an additive in the most diverse galvanic baths, gives a substantial improvement of the brightness, better throwing power, higher permissible current density and, in acid nickel baths, not only excellent brightness but also very considerable leveling effect. From a large number of tests with the esters of selenious acid with a wide variety of alcohols, phenols, thioalcohols and thiophenols, we have found that apparently all the stable selenious acid esters, of which practically only the diesters exist, have the above-mentioned outstanding effects as brighteners in electroplating baths.

By selection of the compounds serving for the esterification and bearing OH or SH groups, by their constitution, and by further substitution, any desirable properties required for any specific electroplating bath can be obtained. Thus, by the introduction of further substituents, for example amino groups, sulpho-acid groups, it is possible to improve the water-solubility of the compounds in the various pH ranges, and with appropriate active groups to, improve the brightening effect for the various metals.

Furthermore, by altering the size and structure of the molecule carrying the esterifiable groups, it is possible to obtain very good properties for the deposited metal coatings. The use of brighteners with high molecular weights according to the invention is advisable in electrolytic baths of the kind in which the metals deposited are not very sensitive to inhibitors, for example zinc and cadmium.

Apart from the selenious acid diesters, known brightening and leveling agents, hardening binders, pore-inhibiting agents, wetting agents and so on may be added to the baths for further improvement and if special effects are required.

It is surprising that even very small quantities of selenious acid diesters give a high effect. Additions of about 0.00005 mol/litre to 0.2 mol/litre are used. In the case of baths for nickel deposition, it is advantageous also to add a small quantity of an acetylene amine.

The following examples illustrate the invention and the manner in which it is carried into effect:

2

## Example 1

Very bright copper precipitates were deposited from a cyanide bath of the following composition:

|   |                                               |          |             |
|---|-----------------------------------------------|----------|-------------|
| 5 | Copper as $\text{Na}_2\text{Cu}(\text{CN})_3$ | g./l...  | 50          |
|   | NaCN (free cyanide)                           | g./l...  | 12          |
|   | Seignette salt                                | g./l...  | 30          |
|   | Dimethyl selenite                             | mol/l... | 0.00005-0.1 |
|   | Polyglycol ether                              | g./l...  | 0.5         |

10 at a bath temperature of 65° C., and with a moving cathode in the current density range from 0.2-3 a./dm.<sup>2</sup>.

Using a 30:1 current-reversal cycle, the bright range is extended to a current density of 5 a./dm.<sup>2</sup>.

## Example 2

Uniform very bright copper deposits were produced on a moving cathode from a cyanide bath of the following composition:

|    |                                               |          |             |
|----|-----------------------------------------------|----------|-------------|
| 20 | Copper as $\text{Na}_2\text{Cu}(\text{CN})_3$ | g./l...  | 60          |
|    | NaCN (free cyanide)                           | g./l...  | 15          |
|    | Sodium citrate                                | g./l...  | 40          |
|    | Bis-(phenolsulfonic acid) selenite            | mol/l... | 0.00005-0.1 |
|    | Polyglycol ether                              | g./l...  | 0.5         |
| 25 | Acid amide sulpho-acids                       | g./l...  | 0.025       |

15 at 70° C., in a current density range from 0.2-4 a./dm.<sup>2</sup>, without current reversal. The cathode current yield is 98-100%.

## Example 3

30 Mirror-bright completely cloud-free silver coatings were obtained from a silver bath of the following composition:

|    |                                                 |          |             |
|----|-------------------------------------------------|----------|-------------|
| 35 | Silver in the form of $\text{KAg}(\text{CN})_2$ | g./l...  | 30          |
|    | KCN (free cyanide)                              | g./l...  | 120         |
|    | $\text{K}_2\text{CO}_3$                         | g./l...  | 40          |
|    | Bis-(2-naphthol-3,6-sulfonic acid) selenite     | mol/l... | 0.00005-0.1 |

40 Turkey red oil

45 and the brightness of these coatings is fully retained even with high coating thicknesses. The resultant silver deposits have a hardness of 140 kg./mm.<sup>2</sup>.

## Example 4

A bath for the deposition of gold has the following composition:

|    |                                             |          |             |
|----|---------------------------------------------|----------|-------------|
| 50 | Gold as $\text{KAu}(\text{CN})_2$           | g./l...  | 3           |
|    | KCN (free cyanide)                          | g./l...  | 100         |
|    | $\text{K}_2\text{HPO}_4$                    | g./l...  | 40          |
|    | Bis-(2-naphthol-3,6-sulfonic acid) selenite | mol/l... | 0.00005-0.1 |

Turkey red oil

55 Very bright gold deposits were obtained at 20-50° C., in current density ranges of 0.1-3 a./dm.<sup>2</sup>.

## Example 5

From a nickel bath of the following composition:

|    |                                               |          |             |
|----|-----------------------------------------------|----------|-------------|
| 60 | $\text{MnSO}_4 \cdot 7\text{H}_2\text{O}$     | g./l...  | 280         |
|    | $\text{NiCl}_2 \cdot 6\text{H}_2\text{O}$     | g./l...  | 40          |
|    | $\text{H}_3\text{BO}_3$                       | g./l...  | 40          |
|    | Benzoic acid sulphimide                       | g./l...  | 1           |
| 65 | Bis-(o-aminophenol-sulphonic acid) diselenite | mol/l... | 0.00005-0.1 |

Lauryl sulphate

70 Acetylene amine

mirror-bright ductile nickel deposits having a good leveling action were obtained at 60° C., in a current density range of 0.1-10 a./dm.<sup>2</sup>.

From the same bath, mirror bright deposits were also

obtained at 20° C., without movement of the article in the current density range from 0.1–2 a./dm.<sup>2</sup>.

*Example 6*

From a nickel bath of the following composition:

|                                      |        |             |
|--------------------------------------|--------|-------------|
| NiSO <sub>4</sub> ·7H <sub>2</sub> O | g./l.  | 280         |
| NiCl <sub>2</sub> ·6H <sub>2</sub> O | g./l.  | 40          |
| H <sub>3</sub> BO <sub>3</sub>       | g./l.  | 40          |
| Naphthalene trisulfonic acid         | g./l.  | 10          |
| Diethyl selenite                     | mol/l. | 0.00005-0.1 |
| Lauryl sulphate                      | g./l.  | 0.5         |
| Acetylene amine                      | g./l.  | 0.015       |

nickel deposits were obtained as in Example 5.

*Example 7*

Very bright zinc deposits were obtained from a cyanidic zinc bath of the following composition:

Zinc as  $\text{Na}_2\text{Zn}(\text{CN})_4$  ----- g./l. 30  
 NaCN (total cyanide) ----- g./l. 50  
 NaOH ----- g./l. 90  
 Diglycerine selenite ----- mol/l. 0.00005-0.1  
 at 20° C., in current density ranges of from 0.1-6 a./dm.<sup>2</sup>

**Example 8**

*Example 8*

Very bright deposits were obtained from a cyanide cadmium bath of the following composition:

|                                                |        |             |
|------------------------------------------------|--------|-------------|
| Cadmium as $\text{Na}_2\text{Cd}(\text{CN})_4$ | g./l.  | 25          |
| NaCN (total cyanide)                           | g./l.  | 100         |
| $\text{NiSO}_4 \cdot 7\text{H}_2\text{O}$      | g./l.  | 1           |
| Di-polyglycol (M.W. 600)<br>selenite           | mol/l. | 0.00005-0.1 |
| Polyglycol ether                               | g./l.  | 1           |

at 20° C., in current density ranges of from 0.5–10 a./dm.<sup>2</sup>, and with cathode movement.

III., and will

1. An aqueous bath for the electrolytic deposition of bright metal coatings, including an ionizable compound of the metal to be deposited, and as a brightener, an effective amount of a stable diester of selenious acid.

2. An aqueous bath for the electrolytic deposition of bright nickel including an ionizable nickel compound and, as a brightener, an effective amount of a stable diester of selenious acid.

### 3. An aqueous bath for the electrolytic deposition of bright nickel including an ionizable nickel compound and

as a brightener, a stable diester of selenious acid in a concentration between 0.00005 and 0.2 mol per liter.

4. An electroplating solution comprising, in aqueous solution, an ionizable compound of a metal to be deposited electrolytically, said solution containing, as a brightener, a stable diester of selenious acid in a concentration between 0.00005 and 0.2 mol per liter.

5. An aqueous electroplating solution comprising a cyanide salt of a metal to be deposited electrolytically, said solution containing, as a brightener, an effective amount of a stable diester of selenious acid.

6. A method of depositing a bright metal coating which comprises electrolyzing an aqueous solution of an ionizable compound of said metal, said solution including an effective amount of a stable diester of selenious acid as a brightener.

7. An electroplating bath comprising an aqueous solution of a source of a metal to be electrodeposited, said source being selected from the group consisting of the complex cyanides of copper, silver, gold, zinc, and cadmium, and the sulfate and chloride of nickel, said solution containing, as a brightener, an effective amount of a stable diester of selenious acid with a compound selected from the group consisting of the lower alkanols, phenosulfonic acid, 2-naphthol-3,6-sulfonic acid, o-aminophenol-sulfonic acid, glycerine, and polyglycol.

8. A method of electrodepositing bright nickel which comprises electrolyzing an aqueous medium containing nickel sulfate, as a source of nickel ions and, as a brightener, an effective amount of a stable diester of selenious acid with a compound selected from the group consisting of the lower alkanols, phenol-sulfonic acid, 2-naphthol-3,6-sulfonic acid, o-aminophenolsulfonic acid, glycerine, and polyglycol.

9. A method as set forth in claim 8, wherein the concentration of said diester in said aqueous medium is between 0.00005 and 0.2 mol per liter.

#### References Cited by the Examiner

UNITED STATES PATENTS

|           |       |          |       |     |      |
|-----------|-------|----------|-------|-----|------|
| 2,701,234 | 2/55  | Wernlund | ----- | 204 | 52.1 |
| 2,770,587 | 11/56 | Ostrow   | ----- | 204 | 52.1 |
| 2,777,810 | 1/57  | Ostrow   | ----- | 204 | 46   |

45 JOHN H. MACK *Primary Examiner*

MURRAY TILLMAN *Examiner*